

1

2,999,751

## CHEMICAL SENSITIZING OF PHOTOGRAPHIC SILVER HALIDE EMULSIONS

Fritz Dersch, Binghamton, N.Y., assignor to General Aniline & Film Corporation, New York, N.Y., a corporation of Delaware  
No Drawing. Filed July 30, 1957, Ser. No. 675,043  
5 Claims. (Cl. 96—107)

This invention relates to photographic materials and 10 particularly to light-sensitive silver halide emulsion containing a reaction product of gelatin and thioformamide as a sensitizing agent for the purpose of increasing the speed and contrast.

Photographic silver halide emulsions are usually prepared by mixing a soluble silver salt such as silver nitrate with a soluble alkali metal halide such as sodium chloride, potassium bromide or potassium iodide in the presence of a colloid, particularly gelatin. The selection of gelatin for this purpose is very critical and requires very careful testing because the photographic properties of the finished emulsion, namely, speed, contrast, freedom from fog and storage stability depend on the presence of minute quantities of active agents in the gelatin. Some of these substances, commonly referred to as ripeners or sensitizers, impart to the emulsion a ripening or sensitizing effect and increase the speed and contrast.

The gelatins with which the emulsion chemist must work are more often than not unsatisfactory because they contain too much or too little of these sensitizers. This is understandable because gelatin is derived from various natural sources including the hides, bones, tendons and sinews of cattle and pigs. Depending on the source of the raw material and on the process selected for the manufacture and extraction, the gelatins will contain varying amounts of these substances.

The nature or chemical structure of the active gelatin ingredients and their actual configuration is far from certain although it is now generally assumed that sulfur containing compounds play a vital part in the natural sensitization of photographic gelatins.

Allyl isothiocyanate, allylthiourea, sodium thiosulfate and sodium polythionates have been suggested in the literature as being the possible photographically active ripening compounds present in the gelatin. It also has been proposed to add these or similar compounds artificially to gelatin or other colloids which serve as gelatin substitutes. However, adding these compounds to gelatin or to photographic emulsions often leads to other complications, particularly the formation of fog so dense that it is beyond control by the usual antifogging agents.

I have found that the reaction products of gelatin and thioformamide possess valuable ripening and sensitizing properties and have the ability, when present in photographic emulsions, to increase their speed, contrast, or both.

The use of the reaction products of gelatin and thioformamide in the preparation of photographic silver halide emulsion, the process of preparing said silver halide emulsions and the silver halide emulsions obtained thereby constitute, accordingly, the purposes and objects of the present invention.

In carrying out the invention, the thioformamide derivative of gelatin is dissolved in water and the resultant solution is added to the gelatin or other colloidal carrier used in the preparation of the emulsion at a stage where the effectiveness of the derivative is most pronounced. In general, this is the case where normally gelatin is added to photographic emulsion. Accordingly, this derivative can be added to the gelatin substitute which is to be used for the initial preparation of the photographic emulsion or it

2

can be used with the gelatin which is added at the ripening stage.

The thioformamide derivatives of gelatin are prepared according to the method described by F. Micheel et al. in "Chemische Berichte," vol. 80, pages 37-38 (1947), and vol. 82, page 136 (1949). It is believed that the reaction product has the following general structure:



The procedure involves reacting 10 parts by weight of an essentially inert gelatin in solid form, preferably powdered or granular, with from 2 to 6 parts by weight of thioformamide which can be used undiluted or as a solution in ether.

Compared with the conventional low molecular ripening agents as illustrated by allyl isothiocyanate or sodium thiosulfate, the gelatin thioformamide reaction product offers the distinct advantage that its available sulfur or sulfide is bound to the gelatin molecule in a manner which bears a strong resemblance to those natural gelatins which have excellent ripening properties. The available sulfur or other ripening body is released gradually and when used in the proper concentrations and conditions does not give rise to the formation of fog.

As mentioned above, the thioformamides are preferably reacted with inert gelatin. Similarly, the reaction products thus obtained are of particular utility when used with inert gelatin. The latter are generally prepared by removing the active agents from a commercially available gelatin, for instance, by prolonged washing or by treatment with charcoal, hydrogen peroxide or peracetic acid as described by H. Ammann-Brass in "Science et Industries Photographiques," vol. 25, page 491 (1954).

The light-sensitive silver salt present in the silver halide materials contemplated herein may be silver bromide, silver iodide, silver chloride or mixed silver halides. The sensitizing silver salt, moreover, may be present in any of the usual photographic carriers or colloids such as gelatin, collodion, albumen, casein, polyvinyl alcohol and the like. In addition, the light-sensitive silver halide materials may contain any of the various ingredients of photographic emulsions, e.g., sensitizing dyes, stabilizers or fog inhibitors, hypersensitizers and surfactants. Finally, the silver halide materials may be those used for producing black and white images or for producing color images particularly those silver halide emulsions which contain a color forming component.

The particular quantities of the thioformamide-gelatin derivatives are critical to the extent that the quantities needed will vary with different types of emulsions. From 20 to 200 milligrams of reaction product per kilogram of colloidal carrier solids have been found most satisfactory. I have further found that optimum results are obtained by utilizing a ratio of silver halide to colloidal carrier to thioformamide on the following order:

60 450 to 750 parts of silver halide  
500 to 1000 parts of the colloidal carrier  
0.02 to 0.2 part of thioformamide gelatin derivative

65 These ratios are expressed in terms of parts by weight. The gelatin thioformamide derivative is water soluble and may, therefore, be incorporated in the emulsion in the form of an aqueous solution. It is also possible to add the derivative in dry form as flakes, powder or shreds to the emulsion.

70 The following examples will further illustrate the invention but it is understood that it is not limited thereto.

## PREPARATION

A reaction product of gelatin with thioformamide is prepared by adding 4 grams of thioformamide to 10 grams of inert gelatin and kneading the mixture thoroughly for six hours until the reaction product is a highly viscous sticky mass. It is washed several times with ether and alcohol in order to remove the excess of thioformamide, and then shaken for two days with alcohol and chloroform and dried. The solid product obtained has a sulfur content of about 4.5 percent.

## Example I

Seventy-five grams of potassium bromide, 4 grams of potassium iodide and 5 grams of gelatin are dissolved in 200 mls. of distilled water. To this solution is added 0.15 cc. of a 0.1 percent solution of the thioformamide gelatin reaction product. The temperature is adjusted to 65° C., and maintained there throughout the mixing operation. A solution of 90 grams of silver nitrate in 800 mls. of water is added to the potassium bromide-iodide gelatin solution over a period of 20 minutes under continuous stirring. At this stage, 100 grams of dry gelatin and 10 mls. of 0.1% solution of the thioformamide gelatin reaction product are added. The mixture is digested for 20 minutes to allow the added gelatin to dissolve. The emulsion is then poured into a shallow pan and allowed to cool. After the emulsion has set to a firm gel, it is cut into cubes and washed, until the inorganic salts are removed. Then the emulsion is re-melted and submitted to another ripening process. During this process, 20 grams dry strength gelatin are added and also 2 cc. of a 0.1% solution of thioformamide treated gelatin. The temperature during the ripening is held at 50° C. The usual coating finals, including stabilizers and surfactants are added and the emulsion is coated on a cellulose ester base and dried.

Samples of these film coatings were then exposed in a Type IIB Sensitometer and developed in a developer of the following composition:

|                                | Grams |
|--------------------------------|-------|
| Metol                          | 1.5   |
| Sodium sulfite, anhydrous      | 45    |
| Sodium bisulfite               | 1     |
| Hydroquinone                   | 3     |
| Sodium carbonate, monohydrated | 6     |
| Potassium bromide              | .8    |
| Water to make 1 liter.         |       |

The developed film was short-stopped, fixed, washed and dried. The film prepared from the emulsion containing the gelatin-thioformamide reaction product was compared with another film prepared and processed in the identical manner except that the thioformamide reaction product had been omitted.

Expressed in numerical terms, the following results were obtained:

|                               | Relative Speed | Gamma | Fog  |
|-------------------------------|----------------|-------|------|
| With thioformamide gelatin    | 100            | 0.85  | 0.08 |
| Without thioformamide gelatin | 15             | 0.15  | 0.06 |

## Example II

Sixty-two grams of silver nitrate are dissolved in 625 mls. of distilled water. Forty-five grams of potassium bromide, 2.2 grams of potassium iodide and 6.25 grams of gelatin are dissolved in 250 cc. of distilled water. 250 cc. of the silver nitrate solution are added with stirring to the bromide-iodide-gelatin solution in one minute and the rest of the silver nitrate solution in 25 minutes. Then 125

grams gelatin dissolved in 300 cc. of water are added and the batch is digested for a period of 25 minutes. The pH of the emulsion is adjusted to 6.8. During the mixing and digestion, the temperature is held at 71° C. The emulsion is then processed as described in Example I and is finally submitted to a second ripening process, for which purpose the washed emulsion is melted slowly, 0.5 gram of the gelatin-thioformamide reaction product are added and the mixture is heated to 40° C. and kept at this temperature for 2 hours. The emulsion is then coated and processed as described in Example I. The results obtained were similar to those described in Example I and the following readings were obtained:

|                                                                 | Relative Speed | Gamma | Fog  |
|-----------------------------------------------------------------|----------------|-------|------|
| Emulsion with the thioformamide gel prepared from inert gelatin | 70             | 0.75  | 0.09 |
| Emulsion without thioformamide gelatin reaction                 | 10             | 0.15  | 0.06 |

Modifications of the invention will occur to persons skilled in the art. I, therefore, do not intend to be limited in the patent granted except as necessitated by the appended claims.

## I claim:

1. The process of increasing the speed of a photographic silver halide emulsion which comprises, digesting an emulsion of silver halide in an essentially inert colloidal carrier in the presence of a sensitizing amount of a reaction product prepared by kneading a mixture of 10 parts by weight of essentially inert solid gelatin and from 2 to 6 parts by weight of thioformamide until a highly viscous sticky mass of reaction product is obtained.
- 35 2. A process as recited in claim 1 wherein the colloidal carrier is gelatin essentially free from natural ripening substances.
3. The process of increasing the speed of a photographic silver halide emulsion which comprises, digesting an emulsion of silver halide in an essentially inert colloidal carrier in the presence of 20 to 200 milligrams per kilogram of said colloidal carrier of a reaction product prepared by kneading a mixture of 10 parts by weight of essentially inert solid gelatin and from 2 to 6 parts by weight of thioformamide until a highly viscous sticky mass of reaction product is obtained.
- 40 4. A process as recited in claim 3 wherein the colloidal carrier is gelatin essentially free from natural ripening substances.
- 45 5. The process of increasing the speed of a photographic silver halide emulsion which comprises, digesting an emulsion of silver halide in an essentially inert colloidal carrier in the presence of a reaction product prepared by kneading a mixture of 10 parts by weight of essentially inert solid gelatin and from 2 to 6 parts by weight of thioformamide until a highly viscous sticky mass of reaction product is obtained, the amount of colloidal carrier in the emulsion ranging from 500 to 1000 parts by weight, the amount of silver halide ranging from 450 to 750 parts by weight and the amount of said reaction product ranging from 0.02 to 0.2 part by weight.

## References Cited in the file of this patent

## UNITED STATES PATENTS

- 65 1,574,944 Sheppard ----- Mar. 2, 1926  
1,623,499 Sheppard et al. ----- Apr. 5, 1927

## OTHER REFERENCES

- 70 Micheel et al.: *Chemische Berichte*, vol. 80, pp. 37-38 (1947).